

Oct. 9, 1934.

C. R. WAGNER

1,976,591

METHOD OF UTILIZING NATURAL HYDROCARBON GASES

Filed March 27, 1930



Inventor  
Cary R. Wagner

By  
W. J. McElroy

Attorney

## UNITED STATES PATENT OFFICE

1,976,591

## METHOD OF UTILIZING NATURAL HYDROCARBON GASES

Cary R. Wagner, Chicago, Ill., assignor to The Pure Oil Company, Chicago, Ill., a corporation of Ohio

Application March 27, 1930, Serial No. 439,468

4 Claims. (Cl. 196—10)

This invention relates to an improved method of utilizing natural hydrocarbon gases. In certain oil producing fields, which are removed from large centers of population, great quantities of natural gas are wasted, since in such fields there is but limited use for gases of this character. In such fields the gas is subjected to compressor recovery operations to extract the liquefiable constituents therefrom and the remaining gases are either burned as fuel or wasted, and it is therefore an outstanding object of the present invention to subject natural gases, of the character referred to, to an economical method of treatment for the purpose of producing therefrom larger percentages of recoverable and liquefiable constituents which are admirably suited for use as motor fuels or as blending stock for motor fuels.

In accordance with the present invention, the latter consists in employing natural gas, or preferably the propane-butane fractions thereof, for the manufacture of a gas containing a high percentage of olefine hydrocarbons, then stripping this latter gas of its liquefiable constituents, and then polymerizing the olefines into motor fuel fractions by regulated heat and pressure conditions.

For a further understanding of the invention reference is to be had to the following description and the accompanying drawing wherein the figure is a diagrammatic view of apparatus employed in carrying the present invention into practical operation.

Referring more particularly to the drawing, the numeral 1 designates a gas storage tank in which is contained ordinary natural gas of the character produced in oil field operations. This gas, or the propane-butane fractions thereof, obtained through the stabilization of natural gas, is withdrawn from the tank 1 and is forced by means of a pump 2 through a cracking coil 3 located within the setting of a tube still or converter 4. The gas while passing through the coil 3 may be maintained under a pressure of between 30 and 50 pounds per square inch and during the passage of the gas through the coil a cracking temperature of between 1200° and 1400° F. is attained thereby. This cracking of the gas results in the production therein of olefines or unsaturated hydrocarbon compounds and the cracked gas contains some liquefiable material of high aromatic content. The gases upon being discharged from the coil 3 pass through a cooler 5 and then into a separator 6 at a pressure of about 30 pounds per square inch. Within the separator the liquefiable constituents, produced

by the cracking operation are removed by way of the pipe line 7 to a storage tank 8.

To further remove the liquefiable constituents from the cracked olefine gases, discharged from the converter 4, the gases which pass overhead from the separator 6 are delivered to a compressor 9 by way of a pipe line 10, and by means of this compressor the gases are placed under super-atmospheric pressure of approximately 200 pounds per square inch by which the cracked gas is deprived to a high degree of its readily liquefiable constituents. From the discharge side of the compressor 9 the recovered liquid constituents, which also contain a high aromatic content, are delivered to the storage tank 8, and may be used there as motor fuels or blending stocks. The gases containing unsaturated hydrocarbons which remain following the compressor operation, as indicated at 9, are then passed to a second pump or compressor 11 wherein the pressure on the gas is increased to approximately 1000 pounds per square inch. Under this latter pressure the gases are passed through a second coil 12 located in the cooler zones of the converter 4, the coil 12 being heated by the furnace gases developed in the converter after such furnace gases have passed over the coil 3 and been deprived of a considerable portion of their heat. Sufficient heat, however, remains in these waste gases to heat the extraneous hydrocarbons passing through the coil 12 to a temperature varying between 500° and 950° F. which, while not cracking the gases in the coil 12 to any material extent, provides for the polymerization of such gases so that a large proportion thereof are changed into additive compounds of higher molecular weight. From the polymerization zone of the still, which is formed by the coil 12, the gases pass into a separator 13 under reduced pressure, there being a pressure reducing valve 14 located in the line 15 extending from the coil 12 to the separator 13. From the bottom of the separator 13 the polymerized compounds are withdrawn and delivered to a storage tank 16 as a motor fuel or as a blending stock for such fuels. The distillate produced in the tank 16 is characterized by its high anti-knock value when used as a fuel for internal combustion engines and, in fact, this anti-knock value is sufficiently high to permit it to be employed as a blending stock for inferior motor fuels which possess a low anti-knock value, to the end that the blended fuels will possess a desired anti-knock rating. The fixed gases discharged from the separator 13 may be economically used as fuel in the operation of various oil

refining processes as, for instance, the present one.

To more fully illustrate the operating conditions surrounding the practical operation of the various steps comprising the present invention, but not to in any way limit the invention, the following examples are given:

*Example 1.*—1000 cubic feet of natural gas when cracked at 1350° F. yielded one gallon of liquid constituents and approximately 1100 cubic feet of gas containing substantially 30% of unsaturated hydrocarbons. This gas when compressed to 1000 pounds pressure and subjected to a temperature of 950° F. yielded two and one-half gallons of liquid material of the boiling range of ordinary gasoline and about 800 cubic feet of dry gas.

*Example 2.*—1000 cubic feet of a mixture of propane and butane cracked at 1300° F., yielded two and one-half gallons of liquid product and about 1700 cubic feet of gas containing approximately 50% of unsaturated hydrocarbons. This gas when compressed to 1000 pounds pressure and subjected to a temperature of 900° F. yielded five gallons of the desired liquid product and approximately 1150 cubic feet of dry gas.

By means of the present invention it is possible to convert 50% or more of the propane-butane fraction of natural gas into an anti-detonating motor fuel of high rating. As stated, the residue gases furnish fuel for the furnace and power for the compressor. In certain oil producing localities the present invention provides for marked economy in that it permits of the utilization of a product which is almost valueless to produce a product that is very much in demand, and possesses a correspondingly high economic value.

What is claimed is:

40. 1. The process for producing low-boiling unsaturated hydrocarbon oils from natural gas, which consists in passing natural gas through a cracking zone, heating the gas during its passage through said zone to conversion temperatures of between 1250° to 1350° F. while said gases are maintained under a pressure of approximately 30 pounds, whereby to produce conversion products comprising a gas containing a high percentage of olefine hydrocarbons and a liquid oil of high aromatic content, removing the olefine gases from said liquid oil and passing the same under a pressure of approximately 200 pounds through a separating zone to remove from said gases its more readily liquefiable constituents, then passing said olefine gases from the separating zone under a pressure of approximately 1000 pounds through a polymerizing zone, wherein said gases are heated to temperatures varying between 500° to 950° F. without substantial cracking, removing the products of the polymerizing zone from said latter

zone, separating the unsaturated low-boiling oils formed therein from the remaining fixed gas, and utilizing the same products of combustion which are employed in the heating of the cracking zone to a high temperature for heating the polymerizing zone to a lower temperature.

2. The method of treating gas composed substantially of hydrocarbons of the methane series which consists in passing the gas through a heating coil in the hotter portion of a furnace wherein the gases are heated to a cracking temperature, passing the cracked gases from the coil to a cooler, compressing the gas to a pressure sufficient to liquefy the normally liquid constituents of the gas without substantially liquefying the normally gaseous portion, separating the liquid portion, further compressing the gas, passing the compressed gas through a heating coil located in a cooler portion of the furnace wherein the gases are heated to a temperature sufficient to induce polymerization but insufficient to cause a substantial amount of cracking and recovering desirable liquid fractions from the vapors issuing from the second heating coil.

3. The method of treating gas composed substantially of hydrocarbons of the methane series which consists in passing the gas through a coil in the hotter portion of a furnace wherein the gas is heated to a temperature of between 1200° and 1400° F. and cracked, cooling the gas and subjecting it to pressure of approximately 200 pounds per square inch whereby the normally liquid constituents are liquefied without substantially liquefying normally gaseous constituents, further compressing the separated gaseous constituents to approximately 1000 pounds per square inch, passing the gas through a second coil located in a cooler zone of the furnace wherein the gas is heated to a temperature of between 500° and 950° F. in order to polymerize the gases without causing substantial cracking, and recovering desirable liquid fractions from the vapors issuing from the second coil.

4. The method of treating gas composed substantially of hydrocarbons of the methane series which consists in passing the gas through a heating coil in the hotter portion of a furnace wherein the gases are heated to a cracking temperature, passing the cracked gases from the coil to a cooler, separating the normally liquefiable constituents from the gaseous portion, and passing the gaseous portion under super-atmospheric pressure through a heating coil located in a cooler portion of the furnace wherein the gases are heated to a temperature sufficient to induce polymerization but insufficient to cause a substantial amount of cracking, and recovering desirable liquid fractions from the vapors issuing from the second heating coil.

CARY R. WAGNER.

135